

Sept. 10, 1940.

W. PEACOCK

2,214,476

METHOD OF MAKING MIRRORS

Filed Oct. 18, 1938



Fig. 2.

*Inventor*

WILLIAM PEACOCK,

*By Leonidelson*  
*Attorney.*

## UNITED STATES PATENT OFFICE

2,214,476

## METHOD OF MAKING MIRRORS

William Peacock, Philadelphia, Pa., assignor, by  
mesne assignments, to Peacock Laboratories,  
Inc., Toledo, Ohio, a corporation of Ohio

Application October 18, 1938, Serial No. 235,661

8 Claims. (Cl. 91—69.1)

This invention relates to an improved method of applying a surface coating or layer of metallic silver which may serve as a reflecting medium when applied to transparent bodies, such as glass, 5 or as a surface decorative medium when applied to translucent or opaque bodies, this application being a continuation in part of my copending application, Serial No. 210,315, filed May 27, 1938. Heretofore and prior to this invention it has 10 been the common practice in the making of mirrors to apply a silvering solution to one surface of a glass while maintaining said surface in a perfectly horizontal plane, the metallic silver being permitted to deposit out of the solution and upon the glass surface. While various expedients have been resorted to in order to insure maintenance of the glass surface in properly leveled condition, this leveling operation nevertheless entails considerable difficulties and the expenditure 15 of much valuable time. Also, in order to insure uniform spreading of the solution over the leveled surface of the glass, such surface must be maintained constantly wetted with the result that the water so present upon the glass surface often interferes with the proper uniform deposition of the silver out of the silvering solution.

In addition, improper leveling of the surface to be silvered results not only in considerable variations in the thickness of the deposited metallic 20 silver film in different areas thereof, the silver film being quite heavy or dense over one area and considerably lighter or thin over another area of the silvered surface, but also in inadequately coated edges.

Moreover, in the conventional methods of silvering mirrors wherein the silvering solution is necessarily poured over the surface to be silvered, it is an exceedingly difficult task to prevent or detect the deposit of non-reflecting decomposition products of the silvering solution along with the reflecting metallic silver. Should these decomposition products be removed during the final rinsing and drying operation, objectionable pin-holes are produced, while should such products 35 perchance remain bound in the silver film, they nevertheless result in translucent spots clearly visible to the eye when the finished mirror is held up to the light.

The present invention has as its object the 40 elimination of the aforementioned objections to and difficulties encountered in the old method of silvering mirrors by the use of separately atomized silver and reducing solutions which may be sprayed onto the glass or other surface while the latter is maintained in a plane inclined at a sub-

stantial angle with respect to the horizontal and which react with sufficient rapidity and degree to insure the deposit of a silver film of a density and homogeneity adequate for mirror purposes.

A further and important object of the present 5 invention is to provide silvering solutions of such formulae that they are suitable for use in atomized state without danger of creating explosive mixtures, it being well known that when accelerating agents, such as sodium or potassium hydroxide are mixed with the usual silver ammonio nitrate solution to form a single mixture a dangerously explosive combination is obtained. To minimize this danger it has been the practice to introduce the caustic alkali at as late a time 10 as possible, the resultant mixture being used without further delay because the explosiveness of the mixture increased with its age. Obviously, this resulted in considerable waste of solutions because unless all of the mixture were employed 15 within a relatively short interval after its preparation, in the interest of safety the unused prepared solutions were required to be destroyed.

In addition, I have found that in order to obtain most satisfactory results by the use of the 20 spray method above set forth, certain compounds, such as hydrazine sulphate, hydrazine hydrate and hydrazine nitrate, serve most effectively as silver reducing agents, and it is among the objects of this invention to provide a method 25 whereby such compounds may be safely employed in conjunction with a caustic soda accelerator in the production of silvered mirrors by the spray method aforesaid.

Other objects and advantages of the invention, 30 such as those relating to economies effected by the use of the hereinafter disclosed method and to the improved character of the silver film or coating so obtained, will be apparent more fully hereinafter.

In the accompanying drawing which illustrates more or less schematically the method of practicing the present invention, Figure 2 illustrates a convenient scheme for supporting a mirror to be silvered in the desired inclined position, 45 while Figure 1 illustrates schematically a solution spraying apparatus for performing the spraying operation.

Referring now more particularly to these figures, it will be observed that the spraying apparatus 50 essentially includes two solution tanks 10 and 11 respectively adapted to contain sprayable solutions A and B which, when mixed together, act to deposit metallic silver upon the surface to be coated. In each instance the silver 55

- solution contains silver nitrate as the principal ingredient, while the reducing agent consists of a hydrazine compound, such as hydrazine sulphate, hydrazine nitrate or hydrazine hydrate.
- 5 While the composition of these solutions may vary, of course, it is preferred that they be produced in accordance with the following exemplary formulae.

Where hydrazine sulphate, nitrate or hydrate 10 is employed in the formulation of the reducing solution, any of the following formulae may be used, it being understood, of course, that in all of the following examples solutions A1 and B1, A2 and B2, etc., are employed conjointly:

15

*Example 1*

|    | Solution A1                                                                                                                                                                                                                                           | Solution B1                                                                                               |
|----|-------------------------------------------------------------------------------------------------------------------------------------------------------------------------------------------------------------------------------------------------------|-----------------------------------------------------------------------------------------------------------|
| 20 | This is preferably a solution of silver ammonio nitrate which is prepared by dissolving 1 oz. of silver nitrate in 100 oz. of distilled water to provide an initial solution into which is added and stirred $\frac{1}{4}$ oz. of ammonium hydroxide. | Solution consisting of 2 oz. of hydrazine sulphate (or nitrate or hydrate) dissolved in 100 oz. of water. |
| 25 |                                                                                                                                                                                                                                                       |                                                                                                           |

*Example 2*

|    | Solution A2                | Solution B2                                                                        |
|----|----------------------------|------------------------------------------------------------------------------------|
| 30 | Same as solution A1 above. | Same as solution B1 above to which is added $\frac{1}{2}$ oz. of sodium hydroxide. |

35

*Example 3*

|    | Solution A3                                           | Solution B3                                                                                                                                          |
|----|-------------------------------------------------------|------------------------------------------------------------------------------------------------------------------------------------------------------|
| 40 | Silver nitrate (1 oz.) dissolved in 100 oz. of water. | Solution consisting of hydrazine sulphate (or nitrate or hydrate) (2 oz.) and ammonium hydroxide ( $\frac{1}{4}$ oz.) dissolved in 100 oz. of water. |

*Example 4*

|    | Solution A4                | Solution B4                                                                        |
|----|----------------------------|------------------------------------------------------------------------------------|
| 45 | Same as solution A3 above. | Same as solution B3 above to which is added $\frac{1}{2}$ oz. of sodium hydroxide. |

50

*Example 5*

|    | Solution A5                                                                                                                           | Solution B5                                                                                   |
|----|---------------------------------------------------------------------------------------------------------------------------------------|-----------------------------------------------------------------------------------------------|
| 55 | Solution consisting of 1 oz. of silver nitrate and 2 oz. of hydrazine sulphate (or hydrate or nitrate) dissolved in 100 oz. of water. | Solution consisting of $\frac{1}{4}$ oz. of ammonium hydroxide dissolved in 100 oz. of water. |

60

*Example 6*

|    | Solution A6                | Solution B6                                                                        |
|----|----------------------------|------------------------------------------------------------------------------------|
| 65 | Same as solution A5 above. | Same as solution B5 above to which is added $\frac{1}{2}$ oz. of sodium hydroxide. |

It is to be understood that in the above formulae for the several solutions A1 and B1, A2 and B2, A3 and B3, etc., the proportions stated 70 are not intended to be critical, are approximate and may be varied within reasonable limits. For example, I have found that by increasing materially the proportion of ammonium hydroxide employed, the speed of reaction between the silver ammonio nitrate and the reducing agent

may be so decreased that an extremely thin or transparent film of silver may be obtained, a result which would have been practically impossible were it not for the control obtained by reducing the speed of reaction. Similarly, other results and effects may be obtained by varying within rather wide limits the proportions of the other ingredients employed. Experience has demonstrated, however, that the above stated proportions produce very desirable results for 10 general purposes.

It is to be observed that in no instance do any of the formulae provide for the mixing together in a single prepared solution silver nitrate and the caustic alkali accelerator, sodium hydroxide. 15 Instead, the solutions respectively containing the silver nitrate and the caustic alkali are always mutually exclusive. In addition, it will be noted that in none of the above formulae is there provided a single prepared solution which commonly contains the silver nitrate, the ammonium hydroxide and the reducing agent. This caustic alkali is employed for the purpose of accelerating the chemical reaction between the silver ammonio nitrate solution and its reducing solution, 20 but where the latter is sufficiently active per se to rapidly effect the deposition of the metallic silver out of the silver solution by reduction of the latter, as in Examples 1, 3 and 5, or where it may be desired to reduce the speed of reaction, 25 the caustic may be dispensed with. In the case of Examples 2, 4 and 6, although the reduction is effected quite rapidly by the hydrazine compound, the caustic alkali is nevertheless employed to still further speed up the reduction, as 30 where the circumstances may require it. In all cases, the caustic alkali may be the sodium hydroxide aforesaid or its equivalent, potassium hydroxide.

In the use of the solutions A and B as above 35 prepared, approximately equal quantities of each are respectively maintained in the containers 10 and 11 in order to insure against the accidental or unintentional exhausting of one solution supply without at the same time exhausting the other, 40 thereby obviating the possibility of spraying only one solution upon the surface to be silvered. Also, where the containers 10 and 11 are supported in elevated position so as to provide a gravity feed for the solutions to the spray gun by 45 maintaining equal solutions in the containers 10 and 11 the maintenance of equal head pressures is insured, thus providing for equalized delivery of the separated solutions to the spray gun.

The spray gun 12 is connected by the conduit 50 13 to a suitable source of compressed air supply, the compressed air being delivered from the gun by way of its discharge nozzle 14, the gun being provided with a suitable air supply control valve not shown) adapted to be operated by a pivoted 55 hand lever 15. Flexible conduits 16 and 17 respectively connected to the tanks 10 and 11, as at 18 and 19, are connected at their forward extremities to suitable fittings 20 and 21 secured at diametrically opposed sides of the compressed air 60 discharge nozzle 14, the fittings 20 and 21 being in communication with the interior of the nozzle 14.

When compressed air is admitted to the spray gun by opening the control valve for the latter, 70 such air passes through and is discharged from the nozzle 14 with suitable velocity. As the compressed air passes the inner open ends of the fittings 20 and 21 the solutions A and B are sucked or drawn out of the tanks 10 and 11 by way of the 75

flexible conduits 16 and 17 and into the air stream where they are atomized and intimately mixed together. While this atomization and intimate mixture of the solutions A and B occurs instantly 5 at the discharge end of the nozzle 14, the resultant reaction of said solutions is not completed before the atomized mixture is brought into contact with the surface to be covered by the metallic silver which is the product of such reaction.

10 Preferably, the flexible conduits 16 and 17 are each provided with suitable valves 22 and 23 conveniently located within reach of the operator of the spray gun, these valves being opened subsequently to the opening of the compressed air control valve in the spray gun. With the valves 15 22 and 23 closed, the supply of the solutions A and B is, of course, interrupted so that only so much of these solutions may be used as is necessary to complete a given silvering operation.

The flexible conduits or tubes 16 and 17 permit independent movement of the spray gun so that it may be readily moved about to direct the discharge therefrom against the proper surface without disturbing the position of the containers 25 10 and 11. In the use of this easily directed spray gun for mirror silvering purposes, the plate glass to be silvered is supported in a position such as is shown in Figure 1. As is therein illustrated, the plate glass 24 is mounted flatwise upon the inclined surface of an easel-like frame 25 which may be suitably supported in any manner upon a table 26. Preferably, the easel 25 is so arranged 30 that its angle of inclination with respect to the horizontal may be varied within wide limits, since it may be desirable in some instances to support the mirror plate 24 in a vertical plane and in other instances in a plane forming an acute angle with the horizontal.

By spraying the silvering material upon the inclined surface of the mirror plate 24, a silver film is obtained of very high quality. Not only is this film of uniformly even thickness throughout but it is more homogeneous due to the substantial absence of pin-holes. Moreover, should any water 45 be present upon the glass surface as would normally tend to interfere with proper deposition of the metallic silver thereupon, it is washed down and thoroughly removed by the force of the spray, directed against the inclined surface of the glass. 50 A further and important advantage of the present method resides in the fact that the solutions A and B may be employed at ordinary room temperatures, in contradistinction to the older methods which usually require heat in the application 55 of the silvering solution.

The present method is particularly adapted for coating with silver other transparent materials such as are obtained from synthetic resins, cellulose derivatives and the like and which ordinarily 60 so deleteriously affect and impair the reaction of the usual silvering solutions applied in the customary manner as to produce unsatisfactory mirrors. Accordingly, it will be understood that the present invention is not limited in its application 65 solely to the silvering of glass for mirror purposes, but instead may be generally employed for providing any surface with a reflective or decorative film of silver, depending upon whether the material, the surface of which is so treated, is 70 transparent or opaque.

What is claimed as new and useful is:

1. A method of coating a surface with a film of metallic silver which comprises directing against said surface a compressed air spray in which are 75 atomized and intimately mixed separately formed

solutions adapted to react with one another to produce metallic silver, one of said solutions containing silver ammonio nitrate and the other of said solutions containing a reducing agent selected from the group consisting of hydrazine sulphate, 5 hydrazine nitrate, and hydrazine hydrate and a caustic alkali accelerator for accelerating the chemical reaction between said solutions.

2. A method of depositing a film of metallic silver upon the surface of a body which comprises 10 preparing and maintaining in separated relation separate solutions of silver ammonio nitrate and a reducing agent therefor, in simultaneously introducing approximately equal quantities of said solution into a jet of compressed air, said solutions being entrained in said jet in the immediate vicinity of its discharge into atmosphere whereby said solutions are atomized and intimately mixed together for reaction to produce metallic silver which is adapted to be applied in the form of a 20 homogeneous film over the surface to be covered, said reducing solution containing an agent selected from the group consisting of hydrazine sulphate, hydrazine nitrate, and hydrazine hydrate 25 and an accelerating caustic alkali.

3. A method of depositing a film of metallic silver upon the surface of a body which comprises preparing and maintaining in separated relation separate solutions of silver ammonio nitrate and a reducing agent therefor, in simultaneously introducing approximately equal quantities of said solution into a jet of compressed air, said solutions being entrained in said jet in the immediate vicinity of its discharge into atmosphere whereby said solutions are atomized and intimately mixed together for reaction to produce metallic silver which is adapted to be applied in the form of a 30 homogeneous film over the surface to be covered, said reducing solution containing a hydrazine compound selected from the group consisting of 35 hydrazine sulphate, hydrazine nitrate, and hydrazine hydrate.

4. A method of forming a metallic silver reflecting film upon a glass or like surface which comprises directing against said surface a compressed air spray in which are atomized and intimately mixed separately formed solutions adapted 45 to react with one another to produce metallic silver, said solutions containing silver nitrate, ammonium hydroxide and a hydrazine compound 50 selected from the group consisting of hydrazine sulphate, hydrazine nitrate, and hydrazine hydrate, at least one of said last-named ingredients being included in a solution separate from that containing the other of said ingredients. 55

5. A method of forming a metallic silver reflecting film upon a glass or like surface which comprises directing against said surface a compressed air spray in which are atomized and intimately mixed separately formed solutions adapted 60 to react with one another to produce metallic silver, said solutions containing silver nitrate, ammonium hydroxide, a reducing agent selected from the group consisting of hydrazine sulphate, 65 hydrazine nitrate and hydrazine hydrate, and an accelerating caustic alkali, at least one of said first three named ingredients being included in a solution separate from that containing the other two of said first three named ingredients, and said caustic alkali being included in the solution other 70 than that containing the silver nitrate.

6. A method of forming a metallic silver reflecting film upon a glass or like surface which comprises directing against said surface a compressed air spray in which are atomized and inti- 75

- mately mixed at least two separately formed solutions adapted to mutually react to produce metallic silver, said solutions containing silver nitrate, ammonium hydroxide, a reducing agent selected from the group consisting of hydrazine sulphate, hydrazine nitrate and hydrazine hydrate and a caustic alkali accelerator and being characterized in that no one of said solutions contains all of the three first named ingredients and further in that the solutions respectively containing the silver nitrate and caustic alkali are mutually exclusive.
7. A method of forming a film of metallic silver upon the surface of a body which comprises mixing in air a liquid spray containing silver ammonio nitrate and a liquid spray containing a reducing agent for said silver ammonio nitrate, and directing said mixed spray against the surface of the body to be covered, the reducing agent being selected from the group consisting of hydrazine sulphate, hydrazine nitrate, and hydrazine hydrate, said metallic silver deposit having a high coefficient of reflection at both the back and front surfaces thereof.

8. A method of forming a film of metallic silver upon the surface of a body which comprises positioning the body so that its surface to be coated is inclined to the horizontal, preparing separate solutions one of which contains silver ammonio nitrate and the other of which contains a reducing agent therefor selected from the group consisting of hydrazine sulphate, hydrazine nitrate, and hydrazine hydrate, mixing in proximity to the surface to be coated a liquid spray of the solution containing silver ammonio nitrate and a liquid spray of the solution containing the reducing agent, and directing said mixed spray against the inclined surface so that the reaction product of said silver ammonio nitrate and reducing agent forms an adherent homogeneous metallic silver deposit thereon having a high coefficient of reflection at both the back and front surfaces thereof, the mixed spray having sufficient force to effect a washing down of the inclined surface being coated.

WILLIAM PEACOCK.